



US007718724B2

(12) **United States Patent**  
**DeCristofaro et al.**

(10) **Patent No.:** **US 7,718,724 B2**  
(45) **Date of Patent:** **May 18, 2010**

(54) **THERMOPLASTIC COMPOSITE MATERIALS FOR WEAR SURFACES AND METHODS FOR MAKING SAME**

(75) Inventors: **John L. DeCristofaro**, Warren Township, NJ (US); **Jason L. DeCristofaro**, Warren Township, NJ (US); **John Anthony Dispensa**, Long Valley, NJ (US); **Leon Klafter**, Brielle, NJ (US); **Richard Thomas LaGrotta**, Livingston, NJ (US)

(73) Assignee: **Alcatel-Lucent USA Inc.**, Murray Hill, NJ (US)

(\*) Notice: Subject to any disclaimer, the term of this patent is extended or adjusted under 35 U.S.C. 154(b) by 238 days.

(21) Appl. No.: **11/717,977**

(22) Filed: **Mar. 14, 2007**

(65) **Prior Publication Data**

US 2008/0226921 A1 Sep. 18, 2008

(51) **Int. Cl.**

**C08K 3/00** (2006.01)  
**B32B 27/36** (2006.01)

(52) **U.S. Cl.** ..... **524/404**; 428/412

(58) **Field of Classification Search** ..... 524/404  
See application file for complete search history.

(56) **References Cited**

U.S. PATENT DOCUMENTS

5,692,875 A \* 12/1997 Boman ..... 414/725  
2002/0187292 A1 \* 12/2002 Singler et al. ..... 428/36.91  
2005/0023112 A1 2/2005 Karnes et al.  
2006/0073004 A1 \* 4/2006 Drexelius et al. ..... 414/719  
2007/0155885 A1 \* 7/2007 Bell et al. ..... 524/430

FOREIGN PATENT DOCUMENTS

EP 1431378 A1 6/2004  
WO WO93/14236 A1 7/1993  
WO WO2005/035642 A1 4/2005

OTHER PUBLICATIONS

Wikipedia, The Free Encyclopedia, Wear, Adhesive Wear, p. 1, <http://en.wikipedia.org/w/index.php?title=Wear&printable=yes>, Last visited Jan. 24, 2007.

Unknown Author, About Wear Strips, Plates and Parts, Global Spec, the Engineering Search Engine, p. 1, [http://motion-controls.globalspec.com/LearnMore/Motion\\_Controls/Linear\\_Rotary\\_Motion\\_Compon...](http://motion-controls.globalspec.com/LearnMore/Motion_Controls/Linear_Rotary_Motion_Compon...), Last visited Jan. 24, 2007.

Wikipedia, The Free Encyclopedia, Molybdenum disulfide, pp. 2, [http://en.wikipedia.org/w/index.php?title=Molybdenum\\_disulfide&printable=yes](http://en.wikipedia.org/w/index.php?title=Molybdenum_disulfide&printable=yes), Last visited Jan. 3, 2007.

Wikipedia, The Free Encyclopedia, Wear, p. 1 <http://en.wikipedia.org/w/index.php?title=Wear&printable=yes>, Last visited Jan. 24, 2007. Zeus, Technical Whitepaper, Friction and Wear of Polymers, pp. 9, 2005.

Unknown Author, Wear Strips, Plates and Parts Engineering Web Results, p. 1 [http://motion-controls.globalspec.com/LearnMore/Motion\\_Controls/Linear\\_Rotary\\_Motion\\_Compon...](http://motion-controls.globalspec.com/LearnMore/Motion_Controls/Linear_Rotary_Motion_Compon...), Last visited Jan. 24, 2007.

Crown Plastics, The Leader in Manufacturing of Thin Gauge UHMW, pp. 2 <http://www.crownplastics.com/UHMW.htm?snti=2-0>, Last visited Jan. 10, 2007.

Delft Outlook, Rocking Rollers, pp. 9, <http://www.delftoutlook.tudelft.nl/info/indexf4fa.html?hoofdstuk=Article&ArtID=5324>, Last visited Jan. 10, 2007.

Whitford Worldwide, Wear, pp. 3, <http://www.whitfordww.com/design/wear.html>, Last visited Jan. 3, 2007.

Devcon Permatex, Protect Surfaces—Sliding Abrasion, p. 1, <http://www.devcon.com/devconcatsoluton.cfm?catide=19>, Last visited Feb. 1, 2007.

ITW Devcon, Part No. 0243, Wear Guard (High Load) Hardener, Material Safety Data Sheet, p. 1, Last revised Jan. 28, 2004, Danvers, MA, US.

ITW Devcon, Part No. 0112, Carbide Putty Resin, Material Safety Data Sheet, p. 1, Last revised Jun. 10, 2004, Danvers, MA, US.

ITW Devcon, Part No. 0200, Putty Hardener 0200, Material Safety Data Sheet, p. 1, Last revised Nov. 15, 2001, Danvers, MA, US.

ITW Devcon, Part No. 0143, Wear Guard (High Load) Resin, Material Safety Data Sheet, p. 1, Last revised Dec. 6, 2001, Danvers, MA, US.

ITW Devcon, Part No. 0239, Wear Guard (Fine Load) Hardener, Material Safety Data Sheet, p. 1, Last revised Dec. 6, 2001, Danvers, MA, US.

Performance Ceramics Company, PCC Ceramic Powders, pp. 2, USA, <http://www.performanceceramics.com/page4.htm>, Last visited Jan. 3, 2007.

PCT Search Report, Search Report and Written Opinion, dated Jun. 13, 2008.

\* cited by examiner

*Primary Examiner*—Ling-Sui Choi

*Assistant Examiner*—Hui Chin

(74) *Attorney, Agent, or Firm*—Fletcher Yoder PC

(57) **ABSTRACT**

The present techniques provide a method for making wear surfaces comprising a thermoplastic matrix blended with ceramic particles. The wear surfaces may optionally contain other materials, such as friction modifying additives. Wear surfaces formed according to these techniques may be used to protect such surfaces as the side rails of conveyor belts, the teeth of buckets used on front end loaders, rock or debris chutes, and self dumping hoppers, among others.





## 1

**THERMOPLASTIC COMPOSITE  
MATERIALS FOR WEAR SURFACES AND  
METHODS FOR MAKING SAME**

**FIELD OF THE INVENTION**

The present invention relates generally to the protection of machinery from wear. More particularly, the invention relates to the use of thermoplastic ceramic composite materials as wear surfaces.

**DESCRIPTION OF THE RELATED ART**

This section is intended to introduce the reader to various aspects of art that may be related to various aspects of the present invention, which are described and/or claimed below. This discussion is believed to be helpful in providing the reader with background information to facilitate a better understanding of the various aspects of the present invention. Accordingly, it should be understood that these statements are to be read in this light, and not as admissions of prior art.

Any surface that is in regular contact with another moving surface is subject to degradation over time, no matter how hard the surface may appear to be. For example, archeologically significant sites may have to be closed to tourist traffic to prevent erosion of the stonework from foot traffic. Degradation from wear is especially apparent in machinery and industrial applications where repetitive movements of one surface across another may cause significant erosion in a short time. A common example is the movement of a piston in a cylinder head in a car engine, which will wear out the engine over time. Even a very small apparent force, such as boxes sliding down a packaging chute, may eventually wear out the rails and surface of the chute. In larger applications, where the stresses are higher, wear may occur more quickly. For example, in mining applications, where heavy ore and rocks are being carried by a conveyor belt, the contact of these materials with the side rails of the conveyor belt may necessitate regular replacement of the rails.

It has been recognized since the late 1960s that there is a significant cost to industrial economies from problems caused by wear. Specific studies have indicated that the economy of the United States may lose several billions of dollars each year in replacement of materials and equipment that have been damaged, or "worn out," by frictional degradation.

Frictional degradation, or wear, may be defined as the process by which interactions of a surface with another surface result in a dimensional loss of the surfaces. The dimensional loss may or may not occur with an actual loss of material. The damaging interaction of the two surfaces is caused by the microscopic roughness of each surface. The high points of each surface are the actual points of contact with the other surface, and are termed "asperites." As one surface is moved across the other surface, the asperites may deform leading to resistance, or friction, in the movement. Further, as the asperites deform they may break off, causing degradation of the surface. Thus, to decrease wear, it is necessary to either harden the asperites to resist deformation or to decrease the interaction between the asperites of the opposing surfaces.

Hardening a surface may involve manufacturing the surface out of an exotic metal alloy. Examples of such alloys may include chromium steel and alloys of titanium, tungsten, or other hard metals. While these alloys may protect the hardened surface from degradation, a softer opposing surface may actually degrade at a faster rate. For this reason, hardening

## 2

may often be confined to protecting parts which are harder to replace, such as ball bearings. Further, if the opposing surface is easier to replace, it may deliberately be made from a softer material to lower the wear on the hardened parts.

5 While effective, hardening a wear surface necessitates creating surfaces or parts out of expensive materials that are, by definition, hard and difficult to work with. For this reason, decreasing the interactions between the two surfaces may be a more economical option.

10 A primary technique for decreasing surface interactions involves lowering the coefficient of friction between two surfaces by the application of lubricating liquids. For example, the use of oil in car engines decreases friction between the surfaces of the pistons and the cylinders, leading to a longer life span for the engine. Without such lubricants, the engine may overheat or the moving parts may gall, i.e., one surface may lose metal to the other surface, leading to catastrophic failure of the engine. While liquid lubricants may commonly be used in machines having moving parts, such as engines or 15 motors, they may not be practical for use with stationary parts across which other materials slide, such as chutes or side rails for conveyor belts.

20 For stationary parts, either hardening the surfaces or producing them from low friction materials may be the only practical choices. However, both of these choices may have significant drawbacks. For example, the use of exotic alloys as surface modifiers in low value applications, such as chutes, may be too expensive for many applications. Furthermore, surfaces made from low friction materials may not be durable enough for practical use.

25 Thermoset plastics may be used to provide more durable low friction coatings for applications in surface protection. However, thermoset plastics are often used in the form of a paste that is spread onto the surface to be protected, forming a permanent bond to the surface. This bonding may limit the reuse of the surface after further wear has occurred, which may force replacement of an entire part. Correct application of a thermoset paste may also require significant time and effort. Furthermore, if the application is performed on the manufacturing site, the equipment may need to be out of service for a significant period of time, further increasing the cost.

**SUMMARY OF THE INVENTION**

30 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 9505 9510 9515 9520 9525 9530 9535 9540 9545 9550 9555 9560 9565 9570 9575 9580 9585 9590 9595 9600 9605 9610 9615 9620 9625 9630 9635 9640 9645 9650 9655 9660 9665 9670 9675 9680 9685 9690 9695 9700 9705 9710 9715 9720 9725 9730 9735 9740 9745 9750 9755 9760 9765 9770 9775 9780 9785 9790 9795 9800 9805 9810 9815 9820 9825 9830 9835 9840 9845 9850 9

Another embodiment provides a front end loader comprising a loader bucket. The loader bucket comprises a blend of one or more types of ceramic particles and a thermoplastic matrix. The ceramic particles comprise at least 50% by volume of the blend.

Another embodiment provides a chute for directing gravity propelled objects to a destination. The chute is comprised of a blend of one or more types of ceramic particles and a thermoplastic matrix. The ceramic particles comprise at least 50% by volume of the blend.

Yet another embodiment provides a self-dumping hopper comprised of a blend of one or more types of ceramic particles and a thermoplastic matrix. The ceramic particles comprise at least 50% by volume of the blend.

#### BRIEF DESCRIPTION OF THE DRAWINGS

Advantages of the invention may become apparent upon reading the following detailed description and upon reference to the drawings in which:

FIG. 1 is a perspective view of an exemplary thermoplastic ceramic composite in accordance with embodiments of the current techniques;

FIG. 2 is a perspective view of a conveyor belt that may use thermoplastic ceramic composites for protection of wear surfaces in accordance with embodiments of the current techniques;

FIG. 3 is a perspective view of a front end loader having a blade and teeth that may be protected by thermoplastic ceramic composites in accordance with embodiments of the present techniques; and

FIG. 4 is a perspective view of a rock or debris chute directing materials into a loader bucket, in which surface of each may be protected by thermoplastic ceramic composites in accordance with embodiments of the present techniques.

#### DETAILED DESCRIPTION OF SPECIFIC EMBODIMENTS

One or more specific embodiments of the present invention will be described below. In an effort to provide a concise description of these embodiments, not all features of an actual implementation are described in the specification. It should be appreciated that in the development of any such actual implementation, as in any engineering or design project, numerous implementation-specific decisions may be made to achieve the developers' specific goals, such as compliance with system-related and business-related constraints, which may vary from one implementation to another. Moreover, it should be appreciated that such a development effort might be complex and time consuming, but would nevertheless be a routine undertaking of design, fabrication, and manufacture for those of ordinary skill having the benefit of this disclosure.

The techniques described in detail below include thermoplastic ceramic composites which may be used for the protection of wear surfaces. These thermoplastic ceramic composites may be made from a blend of a thermoplastic matrix and hard ceramic particles. Optionally, the matrix may also contain friction modifying additives to lower the coefficient of friction of the surface. During wear, the hard ceramic particles embedded in the matrix are exposed, which may protect the thermoplastic matrix and slow further wear. These thermoplastic composites may be formed into any number of protective surfaces for specific applications. The parts made from thermoplastic composite materials may be manufactured off-site and purchased as preformed units for specific

applications. Further, thermoplastic materials may be melted and reformed, which may be advantageous for resurfacing or recycling of a wear surface.

An example of a thermoplastic ceramic composite 10 that may be used for improved resistance to wear, in accordance with embodiments of the current techniques, is shown in FIG. 1. In this perspective view of the thermoplastic ceramic composite 10, the top surface may be used as the wear surface 12. The thermoplastic ceramic composite 10 may be made from a thermoplastic matrix 14 which has embedded ceramic particles 16. The ceramic particles 16 may be a mixture of different sizes and compositions. Further, the thermoplastic ceramic composite 10 may contain friction modifying additives 20 to decrease the coefficient of friction between the thermoplastic ceramic composite 10 and objects that slide across the wear surface 12.

The thermoplastic matrix 14 used to form the thermoplastic ceramic composite 10 may be selected on the basis of the desired surface friction, hardness, or resistance to wear. Thermoplastics that may be used for the thermoplastic matrix 14 include polyolefins, polycarbonates, poly(phenylene sulfides), poly(phenylene oxides), poly(ether ether ketones), polyamides, or combinations thereof. The choice of materials depends on the combination of properties desired. For example, a polyolefin material may have a lower coefficient of friction than a poly(phenylene sulfide), but may also have a lower resistance to damage from heavy objects. Another parameter that may influence the choice of the thermoplastic matrix 14 is the resistance of the matrix to degradation from heat that may be generated by objects sliding across the surface. Accordingly, in applications where heat may be generated, heat resistant thermoplastics such as poly(phenylene sulfide) or poly(ether ether ketone) may be more appropriate than other thermoplastics.

Although the choice of the material for the thermoplastic matrix 14 is an important consideration, the ceramic particles 16 will be the primary component of the wear surface 12 that is in contact with another surface. Thus, the amount and type of ceramic particles 16 in the thermoplastic ceramic composite 10 may significantly affect the properties and life span of the wear surface 12. In embodiments of the present techniques, the ceramic particles 16 may make up as much as 50% of the total composition by volume. In other embodiments, the ceramic particles 16 may make up at much as 90% by volume of the total composition of the thermoplastic ceramic composite 10.

The ceramic particles 16 may be made from alumina, boron carbide, boron nitride, silicon carbide, silicon nitride, magnesium silicate, magnesium oxide, titanium carbide, titanium oxide, tungsten carbide, zirconia, or combinations of these materials. As the thermoplastic ceramic composite 10 is intended to be low cost and easily replaceable, lower cost ceramic materials may be appropriate. Further, the ceramic particles 16 may be comprised of newly manufactured particles or waste particles, such as used alumina sand blasting dust.

The size of the ceramic particles 16 may range from greater than 50 micrometers to less than 1 millimeter. A wide particle size distribution may improve the wear performance of the panel. For example, while larger particles may be less likely to abrade from the matrix, and, thus, more effective at preventing wear, smaller particles may improve the packing efficiency in the matrix. Improved packing of the ceramic particles 16 may lead to a higher concentration of ceramic particles 16 in the thermoplastic matrix 14. This may increase

the number of particles that an opposing surface contacts, which may increase the wear protection of the thermoplastic ceramic composite 10.

The shape of the ceramic particles 16 may also affect the frictional performance of the thermoplastic ceramic composite 10. For example, it may be appropriate to select ceramic particles 16 that are spherical or rod shaped in order to minimize the roughness of the surface of the ceramic particles 16.

Alternatively, the ceramic particles 16 may be flat. These flat particles could be aligned with each other and the wear surface 12 by shear forces during the molding process. The alignment of such flat particles may increase the surface area of ceramic at the wear surface 12, which may increase the wear resistance of the thermoplastic ceramic composite 10.

The ceramic particles 16 may include nanospherical particles, e.g., particles having diameters on the order of 50 to 500 nanometers. These very small particles may decrease the microscopic surface roughness of the thermoplastic ceramic composite 10, which may decrease the overall friction seen as another surface moves across the thermoplastic ceramic composite 10. Further, as the very tiny spherical ceramic particles 16 are worn out of the surface and detach from the thermoplastic matrix, they may act as friction modifying additives 20, as discussed in detail below.

The thermoplastic ceramic composite 10 may contain friction modifying additives 20 to lower the frictional interaction between the wear surface 12 and an opposing surface. Without intending to be limiting, such a decrease in the surface friction may be caused by various interactions between the friction modifying additive 20 and the wear surface 12. For example, the nanospherical particles described above may function as tiny ball bearings, allowing the surfaces to roll across one another. Other friction modifying additives 20 may tend to fill in the surface roughness, lowering the number of asperites available to engage asperites on an opposing surface. Still other additives may lower the adhesion between the surfaces, allowing the surfaces to slide over each other more easily. Examples of materials that may be used as friction modifying additives 20 include graphite, boron powder, calcium carbonate, ground sea shells, talc, rock dust, poly (tetrafluoroethylene) powder, molybdenum sulfide, tungsten sulfide, or combinations of these materials.

The nature and value of the opposing surface may also dictate the choice of the friction modifying additive 20. For example, if the thermoplastic ceramic composite 10 is intended for use in an application wherein rock or other heavy ores are coming in contact with the wear surface 12, a lower cost additive may be appropriate. Alternatively, where a high value surface may contact the thermoplastic ceramic composite 10, a higher cost friction modifying additive 20 may be chosen to protect the opposing surface. This situation may arise, for example, when a chute in a manufacturing facility is used for transporting easily scratched packages.

#### Example of Thermoplastic Ceramic Composite Wear Surface

An embodiment of a thermoplastic ceramic composite 10 made in accordance with the procedures described above was tested for resistance to wear. In this embodiment, a polycarbonate, Lexan® EXL 9330 high impact grade from General Electric, was used as the thermoplastic matrix 14. Approximately 50% by volume of ceramic particles 16 made from randomly sized alumina fragments were blended into this matrix. A comparison sample made from an epoxy matrix containing approximately 50% by volume of randomly sized alumina fragments was also tested. For both samples, the alumina fragments had a mesh up to size six, which corresponds to a wide distribution of particle sizes with a maxi-

mum size of approximate 0.45 mm. The samples contained no friction modifying additives 20.

The testing was performed using a dry sand rubber wheel test, ASTM number G65. In this test, a sample is placed in a frame that pushes the wear surface 12 against a rotating rubber wheel at a constant force. Dry sand is poured from a hopper in between the wear surface 12 and the rubber wheel and is effectively ground into the surface. The dry sand test is usually run for a single time period of 6,000 revolutions. Measurements of the mass of the sample are taken before and after the test, and the density of the material is used to calculate the volume of the sample that is abraded during the test. Conversion of the material loss from mass to volume compensates for different densities, allowing different materials to be compared.

The test procedure described above was modified to minimize the heat exposure by stopping the run after every 1000 revolutions and weighing the samples. Heating of the samples may have distorted the results by melting the polycarbonate matrix, allowing alumina grains to be extracted from the melt. The results obtained from the tests are shown in Table 1.

TABLE 1

#### WEAR SURFACE TEST OF THERMOPLASTIC CERAMIC COMPOSITE

| Matrix Material | No. of Revolutions | Change in Mass (g) | Est. Change in Vol. (ml) |
|-----------------|--------------------|--------------------|--------------------------|
| Polycarbonate   | 1000               | 0.168              | 0.051                    |
|                 | 2000               | 0.005              | 0.002                    |
| Epoxy           | 1000               | 0.239              | 0.072                    |
|                 | 2000               | 0.048              | 0.014                    |
|                 | 3000               | 0.035              | 0.011                    |
|                 | 4000               | 0.017              | 0.005                    |
|                 | 5000               | 0.014              | 0.004                    |

35

The estimated change in volume was calculated on the basis of a composition containing 50% alumina by volume. A density of 3.97 g/ml was used for the alumina, and densities of 1.3 g/ml and 1.2 g/ml were used for the polycarbonate and epoxy, respectively. The testing was stopped after the measured mass dropped below the accurate limits of measurement, around 0.005 g. Accordingly, only two cycles of testing (2000 revolutions) were run on the wear surface 12 having a thermoplastic matrix 14 made from polycarbonate before it dropped below the accurate limits of measurement. In contrast, the epoxy based composite continued to lose a measurable amount of material throughout the test sequence.

#### Applications of Thermoplastic Ceramic Composites

The thermoplastic ceramic composites 10 of the present techniques may be used in any number of applications for improvement of wear resistance. Examples of such applications are shown in FIGS. 2-4, which illustrate a conveyor belt, a front end loader, a rock or debris chute, and a self dumping hopper.

As shown in FIG. 2, a conveyor belt 22 may be used to carry rock fragments 24 in a mining operation. The contact of the rock fragments 24 with the side rails 26 of the conveyor belt 22 may lead to significant wear in a short period of time, necessitating frequent replacement. In embodiments of the present techniques, thermoplastic ceramic composites 10 may be used as wear surfaces 12 to protect the side rails 26. In one embodiment, the side rails 26 may be made from the thermoplastic ceramic composite 10. In another embodiment, the side rails 24 may be metal, with thin panels of the thermoplastic ceramic composites 10 attached to protect the side rails 26.

40

45

50

55

60

65

Another application is shown in FIG. 3, which is a perspective view of a front end loader 28, with a loader bucket 30. The loader bucket 30 is subject to significant wear, especially in heavy service applications such as loading rocks and ores 31. The metal teeth 32 of the loader bucket 30 are a primary site for wear, and must be regularly replaced or resurfaced. In an embodiment of the present techniques, replaceable sheaths 34 made from a thermoplastic ceramic composite 10 may be used to cover the wear surfaces 12 of the metal teeth 32. In another embodiment, the thermoplastic ceramic composite 10 may be formed into teeth that are used in place of the metal teeth 32. Such thermoplastic ceramic composite 10 parts may be easily detached and replaced, minimizing downtime.

In FIG. 4, a chute 36 is used to direct materials 37 into a self-dumping hopper 38. This arrangement may be used, for example, for loading ore in a mining operation or loading construction debris during a demolition operation. The material 37 impacting and sliding along the wear surfaces 12 of the chute 36 and the interior surface 42 of the self-dumping hopper 38 may cause heavy wear, necessitating frequent repair or replacement of the units. In an embodiment of the present techniques, the chute 36 may have panels made from a thermoplastic ceramic composite 10 mounted to the interior wear surfaces 12, protecting these surfaces from damage. Such thermoplastic ceramic composite 10 panels may be easily detached and replaced, minimizing downtime. In another embodiment, the entire chute 36 may be made from thermoplastic ceramic composites 10, which may have both a longer lifespan and a lower cost than a metal chute. Similarly, the self dumping hopper 38 may have panels of the thermoplastic ceramic composite 10 attached to protect the interior surface 42. Alternatively, the self dumping hopper 38 may be made from the thermoplastic ceramic composite 10.

It should be understood that the present techniques have been described above by way of example and that such techniques may apply in other situations as well. Indeed, numerous other applications may take advantage of the enhanced wear, low cost, and recyclability of the thermoplastic ceramic composites 10 discussed above. Examples of such applications may include dumpsters, rolling surfaces for bearings, door jambs, entry mats for buildings, and protective mats for high traffic areas of archeologically valuable tourist attractions, among others.

While the invention may be susceptible to various modifications and alternative forms, specific embodiments have been shown by way of example in the drawings and/or described in detail herein. However, it should be understood that the invention is not intended to be limited to the particular forms disclosed. Rather, the invention is to cover all modifications, equivalents, and alternatives falling within the spirit and scope of the invention as defined by the following appended claims.

We claim:

1. A wear surface of one layer comprising a blend of a thermoplastic matrix and one or more types of ceramic particles, wherein the ceramic particles comprise at least 50% by volume of the blend.

2. The wear surface, as set forth in claim 1, wherein the thermoplastic matrix comprises at least one of a polyolefin, a polycarbonate, a poly(phenylene sulfide), a poly(phenylene oxide), a poly(ether ether ketone), a polyamide, or combinations thereof.

3. The wear surface, as set forth in claim 1, wherein the ceramic particles comprise at least one of alumina, boron carbide, boron nitride, silicon carbide, silicon nitride, magnesium silicate, magnesium oxide, titanium carbide, titanium oxide, tungsten carbide, zirconia, or combinations thereof.

4. The wear surface, as set forth in claim 1, wherein the ceramic particles comprise at least 80% by volume of the blend.

5. The wear surface, as set forth in claim 1, wherein the ceramic particles comprise at least one of random shaped particles, substantially spherical particles, substantially rod shaped particles, substantially flat particles, or combinations thereof.

6. The wear surface, as set forth in claim 1, wherein the ceramic particles comprise substantially flat particles that are aligned substantially parallel to a surface of the structure.

7. The wear surface, as set forth in claim 1, wherein the ceramic particles comprise substantially spherical particles having a diameter greater than about 50 nm and less than about 500 nm.

8. The wear surface, as set forth in claim 1, wherein the ceramic particles comprise a substantially even distribution of sizes from greater than about 0.050 mm to less than about 1 mm.

9. The wear surface, as set forth in claim 1, comprising a protective covering for at least one of a side rail for a conveyor belt, a chute, a debris chute, a rock chute, a bearing surface, a loader bucket, a tooth of a loader bucket, a self dumping hopper, or a dumpster.

10. The wear surface, as set forth in claim 1, comprising at least one of a side rail for a conveyor belt, a chute, a debris chute, a rock chute, a bearing surface, a loader bucket, a tooth of a loader bucket, a self dumping hopper, or a dumpster.

11. The wear surface, as set forth in claim 1, comprising a friction reducing additive.

12. The wear surface, as set forth in claim 11, wherein the friction reducing additive comprises at least one of graphite, poly(tetrafluoroethylene) powder, molybdenum sulfide, tungsten sulfide, boron powder, calcium carbonate, ground seashells, talc, rock dust, or combinations thereof.

13. A method for protecting a surface from wear, comprising blending of one or more types of ceramic particles and a thermoplastic matrix, wherein the ceramic particles comprise at least 50% by volume of the blend; and forming a protective surface from the blend.

14. The method, as set forth in claim 13, wherein the thermoplastic matrix comprises at least one of a polyolefin, a polycarbonate, a poly(phenylene sulfide), a poly(phenylene oxide), a poly(ether ether ketone), a polyamide, or combinations thereof.

15. The method, as set forth in claim 13, wherein the ceramic particles comprise at least one of alumina, boron carbide, boron nitride, silicon carbide, silicon nitride, magnesium silicate, magnesium oxide, titanium carbide, titanium oxide, tungsten carbide, zirconia, or combinations thereof.

16. The method, as set forth in claim 13, wherein the ceramic particles comprise at least 80% by volume of the blend.

17. The method, as set forth in claim 13, wherein the protective surface comprises at least one of a side rail for a conveyor belt, a chute, a debris chute, a rock chute, a bearing surface, a loader bucket, a tooth of a loader bucket, a self dumping hopper, or a dumpster.

18. The method, as set forth in claim 13, wherein the protective surface comprises a protective covering for at least one of a side rail for a conveyor belt, a chute, a debris chute, a rock chute, a bearing surface, a loader bucket, a tooth of a loader bucket, a self dumping hopper, or a dumpster.

19. A conveyor belt comprising a motor driven belt; and side rails on each side of the belt, wherein the side rails comprise a blend of one or more types of ceramic particles

and a thermoplastic matrix, and wherein the ceramic particles comprise at least 50% by volume of the blend.

20. The conveyor belt, as set forth in claim 19, wherein the side rails are made from the blend.

21. The conveyor belt, as set forth in claim 19, wherein the side rails have attached panels comprising the blend.

22. A front end loader comprising a loader bucket, wherein the loader bucket comprises a blend of one or more types of ceramic particles and a thermoplastic matrix, and wherein the ceramic particles comprise at least 50% by volume of the blend.

23. The front end loader, as set forth in claim 22, wherein the loader bucket comprises teeth made from the blend.

24. The front end loader, as set forth in claim 22, wherein the loader bucket comprises teeth having attached covers comprising the blend.

25. A chute for directing gravity propelled objects to a destination comprising a blend of one or more types of

ceramic particles and a thermoplastic matrix, and wherein the ceramic particles comprise at least 50% by volume of the blend.

26. The chute, as set forth in claim 25, comprising attached panels made from the blend.

27. The chute, as set forth in claim 25, wherein the chute is molded from the blend.

28. The chute, as set forth in claim 25, comprising either a rock chute or a debris chute.

10 29. A self-dumping hopper comprising a blend of one or more types of ceramic particles and a thermoplastic matrix, and wherein the ceramic particles comprise at least 50% by volume of the blend.

15 30. The self-dumping hopper, as set forth in claim 29, comprising attached panels made from the blend.

31. The self-dumping hopper, as set forth in claim 29, comprising a hopper bucket made from the blend.

\* \* \* \* \*